

# UNITED STATES PATENT OFFICE.

CHARLES N. FORREST, OF RAHWAY, NEW JERSEY, ASSIGNOR TO THE BARBER ASPHALT PAVING COMPANY, OF PHILADELPHIA, PENNSYLVANIA, A CORPORATION OF WEST VIRGINIA.

## PROCESS OF MANUFACTURING ASPHALTIC PAVING MATERIAL.

1,087,085.

Specification of Letters Patent.

Patented Feb. 10, 1914.

No Drawing.

Application filed January 14, 1910. Serial No. 537,986.

To all whom it may concern:

Be it known that I, CHARLES N. FORREST, a citizen of the United States, residing at Rahway, in the county of Union and State 5 of New Jersey, have invented a certain new and useful Process of Manufacturing Asphaltic Paving Material, of which the following is a specification.

My invention relates to a process for dehydrating crude natural asphalt with formation of an asphaltic cement, as an incident to its incorporation with a suitable mineral aggregate, so as to form a paving mixture for highway or other pavements suitable for 15 motor, horse-drawn or other vehicles.

Asphalt pavements consist of the combination of an asphaltic cementing medium with a suitable mineral aggregate. When natural asphalt such as that from the island 20 of Trinidad, B. W. I., known as lake or land Trinidad asphalt, or from Venezuela, known as Bermúdez asphalt, is employed as the cementing material of a pavement containing also either sand or crushed stone or both, 25 it has heretofore been the practice to first dehydrate the crude natural asphalt by heating it in tanks or stills, by means of either direct fire under the tanks or steam coils inside of the same, to a temperature of approximately 325° F. The dehydrated asphalt prepared thus or in any other way is 30 a relatively hard substance, too hard for direct use in a bituminous pavement mixture. It is therefore softened to a suitable consistency in a fire or steam heated kettle, by 35 adding approximately 20 parts by weight of a heavy petroleum oil to one hundred parts of the dehydrated or so-called refined natural asphalt, after which it is drawn from the 40 fluxing tank in suitable quantities and at convenient times for preparing the paving mixture in conjunction with a hot mineral aggregate. Accordingly the operations customarily employed in the manufacture of 45 asphaltic paving material involve, first, dehydrating the crude asphalt by means of heat, second, fluxing the dehydrated asphalt with heavy petroleum oil by means of heat, and third, incorporating the resulting hot 50 fluxed asphalt cement with a hot mineral aggregate.

My invention consists in a process by which all of the functions of the foregoing three separate operations are performed during one general handling of the materials, 55 and with but one application of heat, and all at the final stage of the operation of preparing by direct composition a suitable paving mixture.

A paving mixture, the mineral aggregate 60 of which consists entirely of sand, (and by sand I mean particles which will pass a wire screen or its equivalent, having eight or ten meshes per lineal inch), contains approximately ten per cent. bitumen and ninety per 65 cent. mineral aggregate. A paving mixture, the mineral aggregate of which is crushed stone, gravel or slag varying in size or entirely of one size from two and one-half inches to eight mesh, will require less 70 than ten per cent. bitumen, the exact amount required depending upon the size, number and shape of said particles of stone in a given volume. In any event the exact amount of bitumen in any pavement mixture, 75 as well as the consistency of the same, is fixed by experience and suitable simple tests well known in the paving art. Crude Trinidad and crude Bermúdez asphalts contain a substantially constant proportion of 80 water, about 29 to 30% in either case, and the exact amount of water present is very readily determined by a simple test.

In order to practise my process after having determined the factors set forth in the 85 last paragraph a suitable proportion calculated by weight upon its bituminous content, of the crude asphalt of either form, is deposited in a pug mill or other suitable mixing device which contains also hot sand, 90 stone or both at a temperature of about 400° F.

The proportions are fixed by a determination of the percentage of asphalt required for the aggregate and that amount of asphalt 95 is employed making allowance for the contained water. Assuming that the crude asphalt is added at atmospheric temperatures, the mineral aggregate heated and proportioned as above explained, will contain 100 a much larger number of heat units than are required to convert into steam substantially

all of the water carried by the crude asphalt.

The result of operating the pug mill is that the asphalt is agitated and thoroughly mixed with the hot mineral aggregate, and the water very quickly and thoroughly driven from the same. A cloud of watery vapor arises from the mixer, but in one or two minutes this ceases and indicates that 10 the asphalt has been completely dehydrated. Thereupon a suitable quantity of heavy petroleum oil of proper quality is added to the mixture of hot sand and asphalt in the mill and agitated for an additional two minutes or more, thus producing the final mixture in suitable form for spreading in the customary manner upon a roadway.

As an example of the proper proportions to be used in an instance where it is proposed to employ crude Trinidad asphalt, let 20 it be supposed that the crude asphalt contains by analysis the following:

|                |        |
|----------------|--------|
| Water          | 29.0%  |
| Bitumen        | 39.0%  |
| Mineral matter | 25.0%  |
| Difference     | 7.0%   |
|                | 100.0% |

30 Under such circumstances, the paving ingredients, for a normal sand mineral aggregate, should be combined as follows:

|                         |            |
|-------------------------|------------|
| Crude Trinidad asphalt. | 18.4 parts |
| Mineral aggregate       | 79.0 "     |
| Heavy petroleum oil     | 2.6 "      |
|                         | 100.0%     |

The result will be that after the dehydration of the crude asphalt and the incorporation of the petroleum oil, the composition of the resulting paving mixture will be approximately 10% bitumen and 90% mineral aggregate.

45 As an example of the proper proportions to be used in an instance where it is proposed to employ crude Bermúdez asphalt, let it be supposed that the Bermúdez asphalt contains by analysis the following:

|                |        |
|----------------|--------|
| Water          | 29.9%  |
| Bitumen        | 68.0%  |
| Mineral matter | 1.1%   |
| Difference     | 1.0%   |
|                | 100.0% |

Under such circumstances, the ingredients for a normal sand mineral aggregate should be combined as follows:

|                        |       |
|------------------------|-------|
| Crude Bermúdez asphalt | 12.7% |
| Mineral aggregate      | 85.6% |
| Heavy petroleum oil    | 1.7%  |

The result will be that after the dehydra-

tion of the crude asphalt and the incorporation of the petroleum oil, the composition of the resulting paving mixture will be approximately bitumen 10.6%, and mineral aggregate 89.4%.

While the above proportions are typical 70 and are approximately correct for a serviceable mixture, it is to be understood that different sands vary as to their capacity for holding asphalt as also does crushed stone. Likewise a mixture for use in a cold climate 75 may require more petroleum oil than one for use in a warm climate. It will, therefore, be understood that my process is not to be limited to any particular proportions of the materials, but includes the immediate 80 combination with a hot mineral aggregate, of a suitable proportion of a crude asphalt calculated upon its bituminous content, so that dehydration of the asphalt is effected by the heat imparted to it during the process 85 of mixing with the hot aggregate, with the result that after dehydration, and the addition of a proper amount of fluxing material, there will remain combined with the aggregate a cementing material of a character and in proportions suitable to the aggregate, with which it is combined, the result being a properly composed paving mixture. It will further be understood that although I propose primarily to utilize the 95 heat of the aggregate for the purpose of effecting dehydration of the crude asphalt, the heat for this purpose, or part of it, may, if desirable, be obtained from other sources and imparted to the mixture. The distinguishing feature of my process is that the dehydration of the crude asphalt is effected as an incident of its mixture with the aggregate with which it is combined for making the paving mixture, as distinguished 100 from former processes where dehydration has been effected at a previous stage of the process, and before the asphalt is mixed with the aggregate.

Having thus described my process, I 110 claim:

1. The process of making a paving mixture which consists in incorporating with crude water containing asphalt, a suitable proportion of a mineral aggregate sufficiently 115 heated to supply the amount of heat required to drive off the water from the crude asphalt, whereby dehydration is effected as an incident to the act of incorporation, and with the result of making a mixture of an 120 aggregate and an asphalt cementing medium in proportions suitable for a paving mixture.

2. The process of making an asphaltic paving mixture, which consists in directly 125 and intimately combining in suitable proportions a hot mineral aggregate, an amount of crude water containing asphalt calculated

upon its bituminous content, and an oil flux, said mineral aggregate being heated hot enough to drive off substantially all of the water contained by the crude asphalt, 5 whereby the crude asphalt is immediately dehydrated and converted into an asphaltic cement, proportioned with reference to the aggregate to form the paving mixture.

In testimony whereof, I have hereunto signed my name, at Maurer, New Jersey, this 12th day of January, 1910.

CHARLES N. FORREST.

Witnesses:

JOHN S. MILLER, Jr.,  
MICHAEL P. ENNIS.

---